

## UNITED STATES PATENT OFFICE

2,330,707

PRODUCTION OF PATTERN EFFECTS ON  
ACETATE RAYONRichard Walter Hardacre, Blackley, Manchester,  
England, assignor to Imperial Chemical In-  
dustries Limited, a corporation of Great BritainNo Drawing. Application September 18, 1941, Se-  
rial No. 411,434. In Great Britain September  
27, 1940

## 3 Claims. (Cl. 8—63)

This invention relates to the production of pattern effects on delusted acetate rayon by a relustering process, and more particularly to the use of certain adipic acid salts in the relustering.

Acetate rayon which has been delusted by means other than insoluble delustering inorganic compounds, e. g. titanium dioxide and barium sulphate, can be relusted by suitable treatment and this treatment when applied locally provides a convenient means of obtaining pattern effects on a delusted ground. One of the most convenient processes which has been used for the purpose is that in which thioglycol S. ( $\text{CH}_2\text{CH}_2\text{OH}$ )<sub>2</sub> is printed on to the delusted material and then steamed. This process, however, has the drawback that the relustering is liable to take place to some extent also on layers of the rayon material adjacent to the printed parts, during the steaming stage of the process.

We have now found that if certain adipic acid salts are used as the relustering agents, there is no liability to the above drawback, and the process is otherwise as convenient as that with thioglycol.

The said salts are water-soluble salts of adipic acid and ammonia or certain amines or pyridine or its derivatives. The amines are alkyl or alkylene derivatives of ammonia including cyclic derivatives, e. g. methylamine, diethylamine, trimethylamine, ethylenediamine, cyclohexylamine, piperidine and hexamethylenetetramine. The pyridine derivatives are its homologues and the technical mixtures sold as pyridine bases. The salts may be either the so-called neutral salts or those having free carboxylic acid or basic radicals as in for instance acid ammonium adipate.

The relustering process of the invention can be employed not only for obtaining an uncoloured lustre on an uncoloured delusted ground, but also for obtaining a coloured lustre on an uncoloured delusted ground, and a lustre on a coloured ground.

Although the invention includes the use of other salts, it appears that excellent results are obtained with ammonium adipate. As ammonia is cheaper and more readily obtainable than the other bases and as it is free from any possible objection as to undesirable odour, it appears that ammonium adipate will be the preferred salt in most cases.

Our invention accordingly consists of a process for the production of pattern effects on acetate rayon which has been delusted by means other than insoluble delustering inorganic compounds, by local relustering, characterised by this that the

relustering is effected by treating with a printing paste containing a salt of adipic acid as hereinbefore defined and if desired a dyestuff for acetate rayon and then steaming.

5 The following examples in which parts are by weight illustrate but do not limit the invention.

## Example 1

10 A printing paste of the following composition is made—

|                                                                   | Parts |
|-------------------------------------------------------------------|-------|
| Ammonium adipate $\text{C}_4\text{H}_8(\text{CO}_2\text{NH}_4)_2$ | 10    |
| Water                                                             | 39    |
| Gum tragacanth thickening (8%)                                    | 51    |
|                                                                   | 100   |

This paste is printed on acetate rayon sateen, which has been delusted by treating with a 1% aqueous soap solution containing 0.2% phenol at 98° C. for 2 hours. The printed material is dried, steamed for half an hour at about 100° C. in a steamer and rinsed in water. An excellent relusted effect is obtained upon a delusted background.

20 25 Instead of using ammonium adipate, a pyridine, methylamine or cyclohexylamine salt of adipic acid may be used with similar results.

## Example 2

30 A printing paste of the following composition is made—

|                                                                          | Parts |
|--------------------------------------------------------------------------|-------|
| Duranol Brilliant Blue BS 1-methylamino-4-hydroxyethylaminoanthraquinone | 4     |
| Ammonium adipate                                                         | 10    |
| Water                                                                    | 26    |
| Nafka Crystal gum thickening (25%)                                       | 60    |
|                                                                          | 100   |

40 The word Nafka is a registered trade-mark. This paste is printed on to a delusted acetate rayon sateen of the kind used in Example 1, and then steamed in a similar way. A blue lustred pattern is thus obtained upon a white matt ground. Without the adipic acid a blue matt effect is obtained.

## Example 3

45 50 This is the same as Example 1 except that the delusted acetate rayon sateen which is used is one which has been dyed with ½% of Duranol Brilliant Blue CB 300 (1,4,5,8-tetraaminoanthraquinone) powder. A relusted blue effect is obtained on a delusted blue ground.

**I claim:**

1. Process for the production of pattern effects on acetate rayon which has been delustered by means other than insoluble delustring inorganic compounds, by local relustering, which comprises printing local areas of said rayon with a paste containing a water soluble salt of adipic acid and then steaming the rayon.

2. Process for the production of pattern effects

on acetate rayon as defined in claim 1 in which said printing paste contains a dyestuff for acetate rayon.

5 3. Process for the production of pattern effects on acetate rayon as defined in claim 1 in which the water-soluble salt of adipic acid is ammonium adipate.

**RICHARD WALTER HARDACRE.**

CERTIFICATE OF CORRECTION.

Patent No. 2,330,707.

September 28, 1943.

RICHARD WALTER HARDACRE.

It is hereby certified that error appears in the printed specification of the above numbered patent requiring correction as follows: Page 1, first column, line 48, for "undesirable" read --undesirable--; and second column, line 34, after "hydroxyethylaminoanthraquinone" insert --paste--; and that the said Letters Patent should be read with this correction there-in that the same may conform to the record of the case in the Patent Office.

Signed and sealed this 9th day of November, A. D. 1943.

Henry Van Arsdale,

Acting Commissioner of Patents.

(Seal)